



US007160653B1

(12) **United States Patent**  
**Huang et al.**

(10) **Patent No.:** **US 7,160,653 B1**  
(45) **Date of Patent:** **Jan. 9, 2007**

(54) **MULTILAYER IMAGEABLE ELEMENT  
CONTAINING EPOXY RESIN**

(75) Inventors: **Jianbing Huang**, Trumbull, CT (US);  
**Shashikant Saraiya**, Fort Collins, CO (US); **Kevin B. Ray**, Fort Collins, CO (US); **Anthony P. Kitson**, Evans, CO (US); **Eugene L. Sheriff**, Carr, CO (US); **Andrew Krebs**, Greeley, CO (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **11/257,864**

(22) Filed: **Oct. 25, 2005**

(51) **Int. Cl.**

**G03F 7/11** (2006.01)  
**G03F 7/14** (2006.01)  
**G03F 7/038** (2006.01)

(52) **U.S. Cl.** ..... **430/15**; 430/281.1; 430/302; 430/905; 430/910; 430/964; 430/271.1

(58) **Field of Classification Search** ..... **430/15**, 430/271.1, 280.1, 302, 905, 910, 964

See application file for complete search history.

(56)

**References Cited**

**U.S. PATENT DOCUMENTS**

|                 |         |                       |
|-----------------|---------|-----------------------|
| 6,152,036 A     | 11/2000 | Verschueren et al.    |
| 6,294,311 B1    | 9/2001  | Shimazu et al.        |
| 6,352,811 B1    | 3/2002  | Patel et al.          |
| 6,352,812 B1    | 3/2002  | Shimazu et al.        |
| 6,358,669 B1    | 3/2002  | Savariar-Hauck et al. |
| 6,528,228 B1    | 3/2003  | Hauck et al.          |
| 6,593,055 B1    | 7/2003  | Shimazu et al.        |
| 2004/0067432 A1 | 4/2004  | Kitson et al.         |
| 2004/0137366 A1 | 7/2004  | Kawauchi et al.       |
| 2005/0037280 A1 | 2/2005  | Loccufier et al.      |

*Primary Examiner*—Richard L. Schilling

(74) *Attorney, Agent, or Firm*—J. Lanny Tucker

(57) **ABSTRACT**

A positive-working imageable element comprises inner and outer layers and a radiation absorbing compound such as an IR absorbing dye. The inner layer includes a polymeric material that is removable using an alkaline developer. An ink receptive outer layer is not removable using an alkaline developer before its exposure to imaging radiation. The outer layer includes a polymer binder having pendant epoxy groups that are substantially unreacted during exposure.

**21 Claims, No Drawings**

**MULTILAYER IMAGEABLE ELEMENT  
CONTAINING EPOXY RESIN**

**FIELD OF THE INVENTION**

This invention relates to positive-working imageable elements having improved shelf life that can be used to form positive-working lithographic printing plates with improved image resolution. It also relates to a method of forming imaged elements from such imageable elements using thermal imaging means.

**BACKGROUND OF THE INVENTION**

In conventional or “wet” lithographic printing, ink receptive regions, known as image areas, are generated on a hydrophilic surface. When the surface is moistened with water and ink is applied, the hydrophilic regions retain the water and repel the ink, and the ink receptive regions accept the ink and repel the water. The ink is transferred to the surface of a material upon which the image is to be reproduced. For example, the ink can be first transferred to an intermediate blanket that in turn is used to transfer the ink to the surface of the material upon which the image is to be reproduced.

Imageable elements useful to prepare lithographic printing plates typically comprise an imageable layer applied over the hydrophilic surface of a substrate. The imageable layer includes one or more radiation-sensitive components that can be dispersed in a suitable binder. Alternatively, the radiation-sensitive component can also be the binder material. Following imaging, either the imaged regions or the non-imaged regions of the imageable layer are removed by a suitable developer, revealing the underlying hydrophilic surface of the substrate. If the imaged regions are removed, the element is considered as positive-working. Conversely, if the non-imaged regions are removed, the element is considered as negative-working. In each instance, the regions of the imageable layer (that is, the image areas) that remain are ink-receptive, and the regions of the hydrophilic surface revealed by the developing process accept water and aqueous solutions, typically a fountain solution, and repel ink.

Imaging of the imageable element with ultraviolet and/or visible radiation is typically carried out through a mask that has clear and opaque regions. Imaging takes place in the regions under the clear regions of the mask but does not occur in the regions under the opaque mask regions. If corrections are needed in the final image, a new mask must be made. This is a time-consuming process. In addition, dimensions of the mask may change slightly due to changes in temperature and humidity. Thus, the same mask, when used at different times or in different environments, may give different results and could cause registration problems.

Direct digital imaging has obviated the need for imaging through a mask and is becoming increasingly important in the printing industry. Imageable elements for the preparation of lithographic printing plates have been developed for use with infrared lasers. Thermally imageable, multi-layer elements are described, for example, U.S. Pat. No. 6,294,311 (Shimazu et al.), U.S. Pat. No. 6,352,812 (Shimazu et al.), U.S. Pat. No. 6,593,055 (Shimazu et al.), U.S. Pat. No. 6,352,811 (Patel et al.), U.S. Pat. No. 6,358,669 (Savarir-Hauck et al.), and U.S. Pat. No. 6,528,228 (Savarir-Hauck et al.), U.S. Patent Application Publication 2004/0067432 A1 (Kitson et al.).

U.S. Patent Application Publication 2005/0037280 (Locufier et al.) describes heat-sensitive printing plate precursors that comprise a phenolic developer-soluble polymer and an infrared radiation absorbing agent in the same layer.

**5 Problem to be Solved**

Multilayer lithographic printing plates usually include an IR-sensitive top layer that is removed using an alkaline developer after imaging. Such top layers can be composed of various phenolic resins such as novolac resins, resole resins, and various hydroxy-substituted acrylates as described for example in the publications noted above.

Imageable elements having topcoats comprising cyclic olefin copolymers are described in copending and commonly assigned U.S. Ser. No. 10/973,799 (filed Oct. 26, 2004). Further, U.S. Patent Application Publication 2004/0137366 (Kawauchi et al.) describes the use of various styrene-maleic anhydride and methacrylate copolymers in the topcoat of imageable elements.

15 Copolymers having pendant carboxy groups are described for use in top layers of heat-sensitive positive-working elements in U.S. Patent Application Publication 2004/0137366 (noted above) to allegedly improve scratch resistance and development latitude. U.S. Pat. No. 6,152,036 (Verschueren et al.) describes the use of hardened epoxy resins in the top layers of positive-working imaging elements. Crosslinking the top layer is said to improve physical and chemical resistance.

20 There is a desire in the industry to provide positive working imaging elements that have high image resolution (or high discrimination between imaged and non-imaged regions). In addition, there is a need for rapid and complete removal of imaged regions and imaging speed. In many instances, what provides one of these properties worsens others. Moreover, there is a need for improved shelf life of imageable elements and improved printing durability of the imaged elements.

**SUMMARY OF THE INVENTION**

25 This invention provides a positive-working imageable element comprising a radiation absorbing compound, and a substrate having thereon, in order:

an inner layer comprising a polymeric material that is removable using an alkaline developer, and

30 an ink receptive outer layer that is not removable using an alkaline developer before its exposure to imaging radiation, that comprises a polymer binder having pendant epoxy groups sufficient to provide an epoxy equivalent weight of from about 130 to about 1000, and that is free of hardener for the pendant epoxy groups.

35 This invention also provides a method for forming an image comprising:

40 A) thermally imaging the positive-working imageable element of the present invention (as described above), thereby forming an imaged element with imaged and non-imaged regions, and

45 B) contacting the imaged element with an alkaline developer to remove only the imaged regions, and

50 C) optionally, baking the imaged and developed element, wherein the imaged element obtained in step A is characterized wherein the pendant epoxy groups in the polymer binder of the outer layer are substantially unreacted.

55 This invention additionally comprises images formed using the method of this invention.

The imageable elements of the present invention contain non-phenolic polymer binders in the outer layer (topcoat) that is not crosslinked but provides improved shelf life, imaging speed, and image resolution of the resulting imaged elements (for example, printing plates). These results are achieved by using an uncrosslinked epoxy-containing polymer in the outer layer that is free of hardener for the pendant epoxy groups.

The imageable elements are particularly suitable for development using a solvent-based alkaline developer including developers that contain a thiosulfate or amino compound as defined below.

#### DETAILED DESCRIPTION OF THE INVENTION

##### Definitions

Unless the context indicates otherwise, when used herein, the terms "imageable element" and "printing plate precursor" are meant to be references to embodiments of the present invention.

In addition, unless the context indicates otherwise, the various components described herein such as "polymeric materials", "epoxy-containing polymer", "phenolic resin binder", "dissolution inhibitor", "added copolymer", "coating solvent", "infrared radiation absorbing compound", "monomeric or polymeric compound comprising a benzoquinone diazide moiety and/or a naphthoquinone diazide moiety", "alkaline developer", and similar terms also refer to mixtures of such components. Thus, the use of the article "a" or "an" is not necessarily meant to refer to only a single component.

Unless otherwise indicated, percentages refer to percents by dry weight.

For clarification of definitions for any terms relating to polymers, reference should be made to "Glossary of Basic Terms in Polymer Science" as published by the International Union of Pure and Applied Chemistry ("IUPAC"), *Pure Appl. Chem.* 68, 2287-2311 (1996). However, any definitions explicitly set forth herein should be regarded as controlling.

Unless otherwise indicated, the term "polymer" refers to high and low molecular weight polymers including oligomers and includes homopolymers and copolymers.

The term "copolymer" refers to polymers that are derived from two or more different monomers. That is, they comprise recurring units having at least two different chemical structures.

The term "backbone" refers to the chain of atoms in a polymer to which a plurality of pendant groups can be attached. An example of such a backbone is an "all carbon" backbone obtained from the polymerization of one or more ethylenically unsaturated polymerizable monomers. However, other backbones can include heteroatoms wherein the polymer is formed by a condensation reaction or some other means.

##### Uses

The imageable elements can be used in a number of ways. The preferred use is as precursors to lithographic printing plates as described in more detail below. However, this is not meant to be the only use of the present invention. For example, the imageable elements can also be used as thermal patterning systems and to form masking elements and printed circuit boards.

##### Imageable Elements

In general, the imageable element of this invention comprises a substrate, an inner layer (also known as an "underlayer"), and an outer layer (also known as a "top layer" or "topcoat") disposed over the inner layer. Before thermal imaging, the outer layer is not removable by an alkaline developer, but after thermal imaging, the imaged regions of the outer layer are removable by the alkaline developer. The inner layer is also removable by the alkaline developer. An infrared radiation absorbing compound (defined below) is preferably present in the inner layer and optionally also in a separate layer between the inner and outer layers.

The imageable elements are formed by suitable application of an inner layer composition to a suitable substrate. This substrate can be an untreated or uncoated support but it is usually treated or coated in various ways as described below prior to application of the inner layer composition. The substrate generally has a hydrophilic surface or at least a surface that is more hydrophilic than the outer layer composition. The substrate comprises a support that can be composed of any material that is conventionally used to prepare imageable elements such as lithographic printing plates. It is usually in the form of a sheet, film, or foil, and is strong, stable, and flexible and resistant to dimensional change under conditions of use so that color records will register a full-color image. Typically, the support can be any self-supporting material including polymeric films (such as polyester, polyethylene, polycarbonate, cellulose ester polymer, and polystyrene films), glass, ceramics, metal sheets or foils, or stiff papers (including resin-coated and metallized papers), or a lamination of any of these materials (such as a lamination of an aluminum foil onto a polyester film). Metal supports include sheets or foils of aluminum, copper, zinc, titanium, and alloys thereof.

Polymeric film supports may be modified on one or both surfaces with a "subbing" layer to enhance hydrophilicity, or paper supports may be similarly coated to enhance planarity. Examples of subbing layer materials include but are not limited to, alkoxy silanes, amino-propyl triethoxysilanes, glycidioxypropyl-triethoxysilanes, and epoxy functional polymers, as well as conventional hydrophilic subbing materials used in silver halide photographic films (such as gelatin and other naturally occurring and synthetic hydrophilic colloids and vinyl polymers including vinylidene chloride copolymers).

A preferred substrate is composed of an aluminum support that may be treated using techniques known in the art, including physical graining, electrochemical graining, chemical graining, and anodizing. Preferably, the aluminum sheet has been subjected to electrochemical graining and is anodized.

An interlayer may be formed by treatment of the aluminum support with, for example, a silicate, dextrose, calcium zirconium fluoride, hexafluorosilicic acid, phosphate/fluoride, poly(vinyl phosphonic acid) (PVPA), vinyl phosphonic acid copolymer, poly(acrylic acid), or acrylic acid copolymer. Preferably, the grained and anodized aluminum support is treated with PVPA using known procedures to improve surface hydrophilicity.

The thickness of the substrate can be varied but should be sufficient to sustain the wear from printing and thin enough to wrap around a printing form. Preferred embodiments include a treated aluminum foil having a thickness of from about 100 to about 600  $\mu\text{m}$ .

The backside (non-imaging side) of the substrate may be coated with antistatic agents and/or slipping layers or a matte layer to improve handling and "feel" of the imageable element.

The substrate can also be a cylindrical surface having the various layer compositions applied thereon, and thus be an integral part of the printing press. The use of such imaged cylinders is described for example in U.S. Pat. No. 5,713,287 (Gelbart).

The inner layer is disposed between the outer layer and the substrate. It is disposed over the substrate and, more typically, disposed directly on the substrate. The inner layer comprises a polymeric material that is removable by the developer and preferably soluble in the developer to reduce sludging of the developer. In addition, the polymeric material is preferably insoluble in the solvent used to coat the outer layer so that the outer layer can be coated over the inner layer without dissolving the inner layer.

Useful polymeric materials for the inner layer include polyvinyl acetals, (meth)acrylic resins comprising carboxy groups, vinyl acetate crotonate-vinyl neodecanoate copolymer phenolic resins, maleated wood rosins, styrene-maleic anhydride co-polymers, (meth)acrylamide polymers, polymers derived from an N-substituted cyclic imide, and combinations thereof. Polymeric materials that provide resistance both to fountain solution and aggressive washes are disclosed in U.S. Pat. No. 6,294,311 (noted above) that is incorporated herein by reference.

Particularly useful polymeric materials include polyvinyl acetals, and copolymers derived from an N-substituted cyclic imide (especially N-phenylmaleimide), a (meth)acrylamide (especially methacrylamide), and a (meth)acrylic acid (especially methacrylic acid). The preferred polymeric materials of this type are copolymers that comprise from about 20 to about 75 mol % and preferably about 35 to about 60 mol % or recurring units derived from N-phenylmaleimide, N-cyclohexylmaleimide, N-(4-carboxyphenyl)maleimide, N-benzylmaleimide, or a mixture thereof, from about 10 to about 50 mol % and preferably from about 15 to about 40 mol % of recurring units derived from acrylamide, methacrylamide, or a mixture thereof, and from about 5 to about 30 mol % and preferably about 10 to about 30 mol % of recurring units derived from methacrylic acid. Other hydrophilic monomers, such as hydroxyethyl methacrylate, may be used in place of some or all of the methacrylamide. Other alkaline soluble monomers, such as acrylic acid, may be used in place of some or all of the methacrylic acid. Optionally, these polymers can also include recurring units derived from (meth)acrylonitrile or N-[2-(2-oxo-1-imidazolidinyl)ethyl]methacrylamide. These polymeric materials are soluble in a methyl lactate/methanol/dioxolane (15:42.5:42.5 wt. % ratio) mixture that can be used as the coating solvent for the inner layer. However, they are poorly soluble in solvents such as acetone and toluene that can be used as solvents to coat the outer layer over the inner layer without dissolving the inner layer.

The bakeable inner layers described in WO 2005/018934 (Kitson et al.) and U.S. Pat. No. 6,893,783 (Kitson et al.), the disclosures of which are all incorporated herein by reference, may also be used.

The inner layer may also comprise one or more primary additional polymeric materials, provided these primary additional polymeric materials do not adversely affect the chemical resistance and solubility properties of the inner layer. Preferred primary additional polymeric materials, when

present, are novolak resins that may be added to improve the run length of the printing member when a post-development bake process is used.

The inner layer may also comprise one or more secondary additional polymeric materials that are resins having activated methylol and/or activated alkylated methylol groups. Such resins include, for example resole resins and their alkylated analogs, methylol melamine resins and their alkylated analogs (for example melamine-formaldehyde resins),  
10 methylol glycoluril resins and alkylated analogs (for example, glycoluril-formaldehyde resins), thiourea-formaldehyde resins, guanamine-formaldehyde resins, and benzoguanamine-formaldehyde resins. Commercially available melamine-formaldehyde resins and glycoluril-formaldehyde resins include, for example, CYMEL® resins (Dyno Cyanimid) and NIKALAC® resins (Sanwa Chemical).

The resin having activated methylol and/or activated alkylated methylol groups is preferably a resole resin or a mixture of resole resins. Resole resins are well known to  
20 those skilled in the art. They are prepared by reaction of a phenol with an aldehyde under basic conditions using an excess of phenol. Commercially available resole resins include, for example, GP649D99 resole (Georgia Pacific) and BKS-5928 resole resin (Union Carbide).

Other useful primary additional polymeric materials include copolymers that comprises from about 1 to about 30 mole % and preferably from about 3 to about 20 mole % of recurring units derived from N-phenylmaleimide, from about 1 to about 30 mole % and preferably from about 5 to about 20 mole % of recurring units derived from methacrylamide, from about 20 to about 75 mole % and preferably from about 35 to about 60 mole % of recurring units derived from acrylonitrile, and from about 20 to about 75 mole % and preferably from about 35 to about 60 mole % of recurring units derived from one or more monomers of the structure:  
30



40 in which R<sub>2</sub> is OH, COOH, or SO<sub>2</sub>NH<sub>2</sub>, and R<sub>3</sub> is H or methyl, and, optionally, from about 1 to about 30 mole % and preferably, when present, from about 3 to about 20 mole % of recurring units derived from one or more monomers of the structure:  
45



in which R<sub>4</sub> is OH, COOH, or SO<sub>2</sub>NH<sub>2</sub>, and R<sub>5</sub> is H or methyl.

50 Useful secondary additional polymeric materials can include copolymers that comprise from about 25 to about 75 mole % and about 35 to about 60 mole % of recurring units derived from N-phenylmaleimide, from about 10 to about 50 mole % and preferably from about 15 to about 40 mole % of recurring units derived from methacrylamide, and from about 5 to about 30 mole % and preferably from about 10 to about 30 mole % or recurring units derived from methacrylic acid. These secondary additional copolymers are disclosed in U.S. Pat. Nos. 6,294,311 and 6,528,228 (both noted above).

60 The polymeric material and the primary and secondary additional polymeric materials useful in the inner layer can be prepared by methods, such as free radical polymerization, that are well known to those skilled in the art and that are described, for example, in Chapters 20 and 21, of *Macromolecules*, Vol. 2, 2nd Ed., H. G. Elias, Plenum, N.Y., 1984. Useful free radical initiators are peroxides such as benzoyl

peroxide, hydroperoxides such as cumyl hydroperoxide and azo compounds such as 2,2'-azobis(isobutyronitrile) (AIBN). Suitable reaction solvents include liquids that are inert to the reactants and that will not otherwise adversely affect the reaction.

In preferred embodiments, the inner layer further comprises an infrared radiation absorbing compound ("IR absorbing compounds") that absorbs radiation at from about 600 to about 1200 and preferably at from about 700 to about 1200 nm, with minimal absorption at from about 300 to about 600 nm. This compound (sometimes known as a "photothermal conversion material") absorbs radiation and converts it to heat. Although one of the polymeric materials may itself comprise an IR absorbing moiety, typically the infrared radiation absorbing compound is a separate compound. This compound may be either a dye or pigment. Examples of useful pigments are ProJet 900, ProJet 860 and ProJet 830 (all available from the Zeneca Corporation).

Useful IR absorbing compounds also include carbon blacks including carbon blacks that are surface-functionalized with solubilizing groups are well known in the art. Carbon blacks that are grafted to hydrophilic, nonionic polymers, such as FX-GE-003 (manufactured by Nippon Shokubai), or which are surface-functionalized with anionic groups, such as CAB-O-JET® 200 or CAB-O-JET® 300 (manufactured by the Cabot Corporation) are also useful.

IR dyes (especially those that are soluble in an alkaline developer) are more preferred to prevent sludging of the developer by insoluble material. Examples of suitable IR dyes include but are not limited to, azo dyes, squarilium dyes, croconate dyes, triarylamine dyes, thioazolium dyes, indolium dyes, oxonol dyes, oxazolium dyes, cyanine dyes, merocyanine dyes, phthalocyanine dyes, indocyanine dyes, indoaniline dyes, merostyryl dyes, indotricarbocyanine dyes, oxatricarbocyanine dyes, thiocyanine dyes, thiaticarbocyanine dyes, merocyanine dyes, cryptocyanine dyes, naphthalocyanine dyes, polyaniline dyes, polypyrrrole dyes, polythiophene dyes, chalcogenopyrrolylidenes and bi(chalcogenopyrrolyl) polymethine dyes, oxyindolizine dyes, pyrylium dyes, pyrazoline azo dyes, oxazine dyes, naphthoquinone dyes, anthraquinone dyes, quinoneimine dyes, methine dyes, arylmethine dyes, squarine dyes, oxazole dyes, croconine dyes, porphyrin dyes, and any substituted or ionic form of the preceding dye classes. Suitable dyes are also described in numerous publications including U.S. Pat. No. 6,294,311 (noted above) and U.S. Pat. No. 5,208,135 (Patel et al.) and the references cited thereon, that are incorporated herein by reference.

Examples of useful IR absorbing compounds include ADS-830A and ADS-1064 (American Dye Source, Baie D'Urfe, Quebec, Canada), EC2117 (FEW, Wolfen, Germany), Cyasorb® IR 99 and Cyasorb® IR 165 (GPTGlendale Inc. Lakeland, Fla.), and IR Absorbing Dye A used in the Examples below.

Near infrared absorbing cyanine dyes are also useful and are described for example in U.S. Pat. No. 6,309,792 (Hauck et al.), U.S. Pat. No. 6,264,920 (Achilefu et al.), U.S. Pat. No. 6,153,356 (Urano et al.), U.S. Pat. No. 5,496,903 (Watanate et al.). Suitable dyes may be formed using conventional methods and starting materials or obtained from various commercial sources including American Dye Source (Canada) and FEW Chemicals (Germany). Other useful dyes for near infrared diode laser beams are described, for example, in U.S. Pat. No. 4,973,572 (DeBoer).

In addition to low molecular weight IR-absorbing dyes, IR dye moieties bonded to polymers can be used as well. Moreover, IR dye cations can be used, that is, the cation is

the IR absorbing portion of the dye salt that ionically interacts with a polymer comprising carboxy, sulfo, phosphor, or phosphono groups in the side chains.

The radiation absorbing compound can be present in the imageable element in an amount of generally at least 12% and up to 30% and preferably from about 12 to about 25%, based on the total inner layer dry weight. The particular amount of a given compound to be used could be readily determined by one skilled in the art.

10 The inner layer can include other components such as surfactants, dispersing aids, humectants, biocides, viscosity builders, drying agents, defoamers, preservatives, antioxidants, and colorants.

15 The inner layer generally has a dry coating coverage of from about 0.5 to about 2.5 g/m<sup>2</sup> and preferably from about 1 to about 2 g/m<sup>2</sup>. The polymeric materials described above generally comprise at least 50 weight % and preferably from about 60 to about 90 weight % based on the total dry layer weight, and this amount can be varied depending upon what other polymers and chemical components are present. Any primary and secondary additional polymeric materials (such as a novolak, resole, or copolymers noted above) can be present in an amount of from about 5 to about 45 weight % and preferably from about 5 to about 25 weight % based on the total dry weight of the inner layer.

20 The outer layer of the imageable element is disposed over the inner layer and in preferred embodiments there are no intermediate layers between the inner and outer layers. The outer layer comprises a polymeric material that is a light-stable, water-insoluble, alkaline developer soluble, film-forming binder material as defined below. The outer layer is substantially free of infrared radiation absorbing compounds, meaning that none of these compounds are purposely incorporated therein and insubstantial amounts diffuse into it from other layers.

25 More particularly, the outer layer comprises one or more polymer binders having pendant epoxy groups sufficient to provide an epoxy equivalent weight of from about 130 to about 1000 (preferably from about 140 to about 750). 30 "Epoxy equivalent weight" refers to the weight of the polymer (grams) divided by the number of equivalence of epoxy groups (number of moles) in the polymer.

35 Any film-forming polymer containing the requisite pendant epoxy groups can be used including condensation polymers, acrylic resins, and urethane resins. The pendant epoxy groups can be part of the polymerizable monomers or reactive components used to make the polymers, or they can be added after polymerization using known procedures. Preferably, the outer layer comprises one or more acrylic resins that are derived from one or more ethylenically unsaturated polymerizable monomers, at least one of which monomers comprises pendant epoxy groups.

40 In preferred embodiments, the outer layer polymer binder can be represented by the following Structure (I)



55 wherein R<sup>1</sup> is hydrogen, a substituted or unsubstituted alkyl group having 1 to 6 carbon atoms (such as methyl, ethyl,

chloromethyl, iso-propyl and benzyl), or a halo group (such as fluoro, chloro, or bromo). Preferably, R<sup>1</sup> is hydrogen, substituted or unsubstituted methyl or chloro, or more preferably, it is hydrogen or unsubstituted methyl.

R<sup>2</sup> represents a substituted or unsubstituted aliphatic or aromatic group containing an epoxy moiety such as a substituted or unsubstituted glycidyl, 3,4-epoxycyclohexylmethyl, or 3,4-epoxyphenyl group. Preferably, R<sup>2</sup> is a glycidyl or 3,4-epoxycyclohexylmethyl group.

L is a direct bond or an aliphatic linking group containing one or more alkylene, arylene, cycloalkylene, or heterocyclic groups connected to each other or to the carbon atom of the polymer backbone with one or more carbonyl, oxy, sulfo, or amido groups.

The substituted or unsubstituted alkylene groups can have 1 to 6 carbon atoms (such as methylene, 1,2-ethylene, 1,1-ethylene, n-propylene, iso-propylene, t-butylene, n-butylene, and n-hexylene groups), substituted cycloalkylene groups can have 5 to 7 carbon atoms in the cyclic ring (such as cyclopentylene and 1,4-cyclohexylene), the substituted or unsubstituted arylene groups can have 6 to 10 carbon atoms in the aromatic ring (such as 1,4-phenylene, naphthylene, 2-methyl-1,4-phenylene, and 4-chloro-1,3-phenylene groups), and the substituted or unsubstituted, aromatic or non-aromatic divalent heterocyclic groups can have 5 to 10 carbon and one or more heteroatoms (nitrogen, oxygen, or sulfur atoms) in the cyclic ring (such as pyridylene, pyrazylene, pyrimidylene, or thiazolylenes groups). Combinations of two or more of these divalent linking groups can be used.

Preferably, L represents a carboxylic acid ester group such as a substituted or unsubstituted —C(O)O-alkylene, —C(O)O-alkylene-phenylene-, or —C(O)O-phenylene group wherein alkylene has 1 to 4 carbon atoms. More preferably, L is a —C(O)O-alkylene, —C(O)O-alkylene-phenylene-, or —C(O)O-phenylene group and most preferably, it is a —C(O)O-alkylene group wherein the alkylene group has 1 or 2 carbon atoms.

Preferred ethylenically unsaturated polymerizable monomers having pendant epoxy groups useful in to make these polymer binders include glycidyl acrylate, glycidyl methacrylate, 3,4-epoxycyclohexyl methacrylate, and 3,4-epoxycyclohexyl acrylate. Mixtures of these monomers can also be used to make the polymer binders.

In Structure (I) noted above, B represents recurring units derived from one or more ethylenically unsaturated polymerizable monomers that do not have pendant epoxy groups. A person skilled in the art would know which monomers would be useful in this context but particularly useful classes of monomers include, but are not limited to, (meth)acrylates, (meth)acrylamides, vinyl ether, vinyl esters, vinyl ketones, olefins, unsaturated imides (such as maleimide), N-vinyl pyrrolidones, N-vinyl carbazole, vinyl pyridines, (meth)acrylonitriles, and styrenic monomers. Of these, the (meth)acrylates, (meth)acrylamides, and styrenic monomers are preferred and the styrenic monomers are most preferred.

Mixtures of monomers can be used to provide a mixture of recurring units represented by "B" in Structure (I). For example, a styrenic monomer could be used in combination with methacrylamide, acrylonitrile, maleimide, vinyl acetate, or N-vinyl pyrrolidone.

Further, in Structure (I), x is from about 20 to 100 weight %, preferably from about 40 to about 95 weight %, and more preferably from about 50 to about 80 weight %. In addition,

y is from 0 to about 80 weight %, preferably from about 5 to about 60 weight %, and more preferably from about 20 to about 50 weight %.

In preferred embodiments, the element has a polymer binder having from about 50 to about 80 weight % of recurring units that are derived from one or more of glycidyl acrylate, glycidyl methacrylate, 3,4-epoxycyclohexyl methacrylate, and 3,4-epoxycyclohexyl acrylate, and at least some recurring units derived from one or more styrenic monomers.

The polymer containing pendant epoxy groups used in the outer layer can be prepared by conventional condensation or addition polymerization methods depending upon the type of polymer to be used. The starting materials and reaction conditions would be readily apparent to one skilled in the polymer chemistry art. Representative synthetic methods are provided below before the Examples.

Generally, the polymer having pendant epoxy groups described above comprises from about 20 to about 99.9 weight %, preferably from about 45 to about 95 weight %, and more preferably from about 65 to about 90 weight %, of the total dry weight of the outer layer.

The outer layer is free of compounds that act as hardeners for the pendant epoxy groups. This means that such compounds are present in the outer layer in amount of less than 0.5 weight %, or in amounts insufficient to provide appreciable hardening (or ring opening) of the polymer epoxy groups. Thus, the pendant epoxy groups are substantially unreacted during exposure of the imageable element. By "substantially", we mean that less than 20% of the epoxy groups are reacted (for example with a hardener or other chemical reaction) during exposure of the imageable element.

It may be possible for the outer layer to further include a monomeric or polymeric compound that includes a benzoquinone diazide and/or naphthoquinone diazide moiety such as phenolic resins that are derivatized with a benzoquinone diazide and/or naphthoquinone diazide moiety as described for example in U.S. Pat. No. 5,705,308 (West et al.) and U.S.

Pat. No. 5,705,322 (West et al.) that are incorporated by reference. Mixtures of such compounds can also be used. An example of a useful polymeric compound of this type is P-3000, a naphthoquinone diazide of a pyrogallol/acetone resin (available from PCAS, France). Other useful compounds containing diazide moieties are described for example in U.S. Pat. No. 6,294,311 (noted above) and U.S. Pat. No. 5,143,816 (Mizutani et al.) that are incorporated by reference.

The outer layer can optionally include colorants. Particularly useful colorants are described for example in U.S. Pat. No. 6,294,311 (noted above) including triarylmethane dyes such as ethyl violet, crystal violet, malachite green, brilliant green, Victoria blue B, Victoria blue R, and Victoria pure blue BO. These compounds can act as contrast dyes that distinguish the unimaged areas from the imaged areas in the developed imageable element.

When a colorant is present in the outer layer, its amount can vary widely, but generally it is present in an amount of at least 0.1 weight % and up to 30 weight %, and preferably from about 0.2 to about 5 weight %, based on the total dry weight of the outer layer.

The outer layer can optionally also include contrast dyes, printout dyes, coating surfactants, dispersing aids, humectants, biocides, viscosity builders, drying agents, defoamers, preservatives, and antioxidants. Coating surfactants are particularly useful.

## 11

Thus, a particularly useful outer layer composition includes about 99 weight % of one or more of the epoxy-containing polymers described above, about 0.3 weight % of a colorant, and about 0.7 weight % of a coating surfactant, all based on total dry weight of the outer layer.

The outer layer generally has a dry coating coverage of from about 0.2 to about 1 g/m<sup>2</sup> and preferably from about 0.4 to about 0.7 g/m<sup>2</sup>.

Although not preferred, there may be a separate layer that is in between and in contact with the inner and outer layers. This separate layer can act as a barrier to minimize migration of radiation absorbing compound(s) from the inner layer to the outer layer. This separate "barrier" layer generally comprises a polymeric material that is soluble in the alkaline developer. If this polymeric material is different from the polymeric material(s) in the inner layer, it is preferably soluble in at least one organic solvent in which the inner layer polymeric materials are insoluble. A preferred polymeric material of this type is a poly(vinyl alcohol). Generally, this barrier layer should be less than one-fifth as thick as the inner layer, and preferably less than one-tenth as thick as the inner layer.

## Preparation of the Imageable Element

The imageable element can be prepared by sequentially applying an inner layer formulation over the surface of the substrate (and any other hydrophilic layers provided thereon), and then applying an outer layer formulation over the inner layer using conventional coating or lamination methods. It is important to avoid intermixing the inner and outer layer formulations.

The inner and outer layers can be applied by dispersing or dissolving the desired ingredients in a suitable coating solvent, and the resulting formulations are sequentially or simultaneously applied to the substrate using suitable equipment and procedures, such as spin coating, knife coating, gravure coating, die coating, slot coating, bar coating, wire rod coating, roller coating, or extrusion hopper coating. The formulations can also be applied by spraying onto a suitable support (such as an on-press printing cylinder).

The selection of solvents used to coat both the inner and outer layers depends upon the nature of the polymeric materials and other components in the formulations. To prevent the inner and outer layer formulations from mixing or the inner layer from dissolving when the outer layer formulation is applied, the outer layer formulation should be coated from a solvent in which the polymeric materials of the inner layer are insoluble. Generally, the inner layer formulation is coated out of a solvent mixture of methyl ethyl ketone (MEK), 1-methoxypropan-2-ol,  $\gamma$ -butyrolactone, and water, a mixture of diethyl ketone (DEK), water, methyl lactate, and  $\gamma$ -butyrolactone, a mixture of DEK, water, and methyl lactate, or a mixture of methyl lactate, methanol, and dioxolane. The outer layer formulation is generally coated out of DEK or a mixture of DEK and 1-methoxy-2-propyl acetate.

Alternatively, the inner and outer layers may be applied by conventional extrusion coating methods from melt mixtures of the respective layer compositions. Typically, such melt mixtures contain no volatile organic solvents.

Intermediate drying steps may be used between applications of the various layer formulations to remove solvent(s) before coating other formulations. Drying steps may also help in preventing the mixing of the various layers.

Representative methods for preparing imageable elements of this invention are shown in Examples 1-6 below.

## 12

The imageable elements can have any useful form including, but not limited to, printing plate precursors, printing cylinders, printing sleeves and printing tapes (including flexible printing webs). Preferably, the imageable members are printing plate precursors useful for providing lithographic printing plates.

Printing plate precursors can be of any useful size and shape (for example, square or rectangular) having the requisite inner and outer layers disposed on a suitable substrate. Printing cylinders and sleeves are known as rotary printing members having the substrate and inner and outer layers in a cylindrical form. Hollow or solid metal cores can be used as substrates for printing sleeves.

## 15 Imaging and Development

During use, the imageable element is exposed to a suitable source of infrared using an infrared laser at a wavelength of from about 600 to about 1200 nm and preferably from about 700 to about 1200 nm. The lasers used to expose the imaging members of this invention are preferably diode lasers, because of the reliability and low maintenance of diode laser systems, but other lasers such as gas or solid state lasers may also be used. The combination of power, intensity and exposure time for laser imaging would be readily apparent to one skilled in the art. Presently, high performance lasers or laser diodes used in commercially available imagesetters emit infrared radiation at a wavelength of from about 800 to about 850 nm or from about 1040 to about 1120 nm.

The imaging apparatus can function solely as a platesetter or it can be incorporated directly into a lithographic printing press. In the latter case, printing may commence immediately after imaging, thereby reducing press set-up time considerably. The imaging apparatus can be configured as a flatbed recorder or as a drum recorder, with the imageable member mounted to the interior or exterior cylindrical surface of the drum. Examples of useful imaging apparatus are available as models of Creo Trendsetter® imagesetters available from Creo Corporation (a subsidiary of Eastman Kodak Company, Burnaby, British Columbia, Canada) that contain laser diodes that emit near infrared radiation at a wavelength of about 830 nm. Other suitable imaging sources include the Gerber Crescent 42T Platesetter that operates at a wavelength of 1064 nm (available from Gerber Scientific, Chicago, Ill.) and the Screen PlateRite 4300 series or 8600 series platesetter (available from Screen, Chicago, Ill.). Additional useful sources of radiation include direct imaging presses that can be used to image an element while it is attached to the printing plate cylinder. An example of a suitable direct imaging printing press includes the Heidelberg SM74-DI press (available from Heidelberg, Dayton, Ohio).

Imaging speeds may be in the range of from about 50 to about 1500 mJ/cm<sup>2</sup>, and more particularly from about 75 to about 400 mJ/cm<sup>2</sup>.

While laser imaging is preferred in the practice of this invention, imaging can be provided by any other means that provides thermal energy in an imagewise fashion. For example, imaging can be accomplished using a thermoresistive head (thermal printing head) in what is known as "thermal printing", as described for example in U.S. Pat. No. 5,488,025 (Martin et al.) and as used in thermal fax machines and sublimation printers. Thermal print heads are

## 13

commercially available (for example, as Fujitsu Thermal Head FTP-040 MCS001 and TDK Thermal Head F415 HH7-1089).

In any case, imaging is generally carried out by direct digital imaging. The image signals are stored as a bitmap data file on a computer. Such files may be generated by a raster image processor (RIP) or other suitable means. The bitmaps are constructed to define the hue of the color as well as screen frequencies and angles.

10 Imaging of the imageable element produces an imaged element that comprises a latent image of imaged (exposed) and non-imaged (non-exposed) regions. Developing the imaged element with a suitable alkaline developer removes the exposed regions of the outer layer and the underlying layers (including the inner layer), and exposing the hydrophilic surface of the substrate. Thus, the imageable elements of this invention are "positive-working". The exposed (or imaged) regions of the hydrophilic surface repel ink while the unexposed (or non-imaged) regions of the outer layer accept ink.

15 More particularly, development is carried out for a time sufficient to remove the imaged (exposed) regions of the outer layer and underlying layers, but not long enough to remove the non-imaged (non-exposed) regions of the outer layer. Thus, the imaged (exposed) regions of the outer layer are described as being "soluble" or "removable" in the alkaline developer because they are removed, dissolved, or dispersed within the alkaline developer more readily than the non-imaged (non-exposed) regions of the outer layer. Thus, the term "soluble" also means "dispersible".

20 The imaged elements are generally developed using conventional processing conditions. Both aqueous alkaline developers and solvent-based alkaline developers can be used with the latter type of alkaline developers being preferred.

25 Aqueous alkaline developers generally have a pH of at least 7 and preferably of at least 11. Useful alkaline aqueous developers include 3000 Developer, 9000 Developer, GOLDSTAR Developer, GREENSTAR Developer, ThermalPro Developer, PROTHERM Developer, MX1813 Developer, and MX1710 Developer (all available from Kodak Polychrome Graphics, a subsidiary of Eastman Kodak Company). These compositions also generally include surfactants, chelating agents (such as salts of ethylenediaminetetraacetic acid), and alkaline components (such as inorganic metasilicates, organic metasilicates, hydroxides, and bicarbonates).

30 Solvent-based alkaline developers are generally single-phase solutions of one or more organic solvents that are miscible with water. Useful organic solvents the reaction products of phenol with ethylene oxide and propylene oxide [such as ethylene glycol phenyl ether (phenoxyethanol)], benzyl alcohol, esters of ethylene glycol and of propylene glycol with acids having 6 or less carbon atoms, and ethers of ethylene glycol, diethylene glycol, and of propylene glycol with alkyl groups having 6 or less carbon atoms, such as 2-ethylethanol and 2-butoxyethanol. The organic solvent(s) is generally present in an amount of from about 0.5 to about 15% based on total developer weight. It is particularly desirable that the alkaline developer contain one or more thiosulfate salts or amino compounds that include an alkyl group that is substituted with a hydrophilic group such as a hydroxy group, polyethylene oxide chain, or an acidic group having a pKa less than 7 (more preferably less than 5) or their corresponding salts (such as carboxy, sulfo, sulfonate, sulfate, phosphonic acid, and phosphate groups). Particularly useful amino compounds of this type include,

## 14

but are not limited to, monoethanolamine, diethanolamine, glycine, alanine, aminoethylsulfonic acid and its salts, aminopropylsulfonic acid and its salts, and Jeffamine compounds (for example, an amino-terminated polyethylene oxide).

5 Representative solvent-based alkaline developers include ND-1 Developer, 955 Developer and 956 Developer (available from Kodak Polychrome Graphics, a subsidiary of Eastman Kodak Company), and the TSD-01 Developer described below. The TSD-01 and ND-1 Developers are particularly useful.

10 Generally, the alkaline developer is applied to the imaged element by rubbing or wiping the outer layer with an applicator containing the developer. Alternatively, the imaged element can be brushed with the developer or the developer may be applied by spraying the outer layer with sufficient force to remove the exposed regions. Still again, the imaged element can be immersed in the developer. In all 15 instances, a developed image is produced, particularly in a lithographic printing plate, having excellent resistance to press room chemicals.

20 Following development, the imaged element can be rinsed with water and dried in a suitable fashion. The dried element can also be treated with a conventional gumming solution (preferably gum arabic).

25 The imaged and developed element can also be baked in a postbake operation that can be carried out to increase run 30 length of the resulting imaged element. Baking can be carried out, for example at from about 220° C. to about 240° C. for from about 7 to about 10 minutes, or at about 120° C. for 30 minutes.

35 Printing can be carried out by applying a lithographic ink and fountain solution to the printing surface of the imaged element. The ink is taken up by the non-imaged (non-exposed or non-removed) regions of the outer layer and the fountain solution is taken up by the hydrophilic surface of the substrate revealed by the imaging and development process. The ink is then transferred to a suitable receiving 40 material (such as cloth, paper, metal, glass, or plastic) to provide a desired impression of the image thereon. If desired, an intermediate "blanket" roller can be used to transfer the ink from the imaged member to the receiving material. The imaged members can be cleaned between 45 impressions, if desired, using conventional cleaning means and chemicals.

50 The following examples are provided to illustrate the practice of the invention but are by no means intended to limit the invention in any manner.

## EXAMPLES

55 The components and materials used in the examples and analytical methods were as follows:

MEK is methyl ethyl ketone.

DEK is diethyl ketone.

60 PGME is 1-methoxypropan-2-ol. It is also known as Dowanol PM.

BLO is  $\gamma$ -butyrolactone.

65 D11 dye is ethanaminium, N-[4-[[4-(diethylamino)phenyl][4-(ethylamino)-1-naphthalenyl]methylene]-2,5-cyclohexadien-1-ylidene]-N-ethyl-, salt with 5-benzoyl-4-hydroxy-2-methoxybenzenesulfonic acid (1:1) as supplied by PCAS (Longjumeau, France).



IR Dye A is an infrared absorbing dye was obtained from Honeywell (Morristown, N.J.).



IR dye B is Kayasorb PS210CnE, an infrared absorbing dye as supplied by Nippon Kayaku Co, Ltd. (Tokyo, Japan).

IR absorbing Dye C was obtained from Eastman Kodak Company and is represented by the following formula:



ACR-1478 is a copolymer having recurring units derived from N-phenylmaleimide (41.5 mol %), methacrylamide (37.5 mol %), and methacrylic acid (21 mol %).

JK69 is a copolymer having recurring units derived from N-phenylmaleimide (40 mol %), methacrylamide (35 mol %), and methacrylic acid (25 mol %).

Ethyl violet is C.I. 42600 (CAS 2390-59-2,  $\gamma_{max}$ =596 nm) having a formula of  $(p\text{-(CH}_3\text{CH}_2\text{)}_2\text{NC}_6\text{H}_4\text{)}_3\text{C}^+\text{Cl}^-$  (Aldrich Chemical Company, Milwaukee, Wis., USA).

TSD01 is a developing solution ("developer") formulated with water (726.39 g), monoethanolamine (6.64 g), diethanolamine (99%, 34.44 g), Pelex NBL (35%, 177.17 g), and

benzyl alcohol (55.36 g). Pelex NBL is available from the Kao Corporation (Tokyo, Japan).

Byk® 307 is a polyethoxylated dimethylpolysiloxane copolymer that is available from Byk Chemie (Wallingford, Conn.) in a 25 wt. % xylene/methoxypropyl acetate solution.

Substrate A was a 0.3 mm gauge aluminum sheet that had been electro-grained, anodized, and subjected to treatment with poly(vinyl phosphonic acid).

ND-1 is a solvent-based developer available from Kodak 10 Polychrome Graphics (Norwalk, Conn., USA, a subsidiary of Eastman Kodak Company).

Epon 1001F is a bisphenol A epoxy resin that is available from Resolution Performance Products (Houston, Tex.).

2-Methylimidazole is a hardener for epoxy resins (as described in U.S. Pat. No. 6,152,036, noted above) that is available from Aldrich Chemical Company (Milwaukee, Wis.).

The following epoxy-containing polymers were prepared and used in the Examples below:

#### Synthesis of Polymer A(1) & A(2):

Into a 1-liter four-neck flask equipped with a heating mantle, thermometer, air powered stirrer, water cooled reflux condenser, Claisen adapter (Corning 9040 Ace Glass # 4015), and a nitrogen sweep were placed 506.62 grams of 1,3-dioxolane, 16.99 grams of styrene, 23.19 grams of glycidyl methacrylate, and 0.84 grams of 1-dodecanethiol.

TABLE I

| Compound              | Molar Ratio | Weight % | Amount (g) |
|-----------------------|-------------|----------|------------|
| Styrene               | 49.375      | 41.42    | 16.99      |
| Glycidyl methacrylate | 49.375      | 56.54    | 23.19      |
| 1-Dodecanethiol       | 1.25        | 2.04     | 0.84       |

This reaction solution was stirred and warmed to reflux (about 65–70° C.) under a nitrogen sweep for one hour. Then, 0.70 grams of a 5% (wt/wt) solution of N,N'-azobis (isobutyronitrile) (AIBN) dissolved in 1,3-dioxolane was 35 added every hour for 20 hours. The reaction solution was then concentrated at ambient pressure to approximately 1/3 to 1/2 volume and cooled. The resulting solution was poured with good stirring into cold methanol, collected, rinsed with cold methanol, collected, and dried at 40° C. at ambient 40 pressure to recover Polymer A(1) (Batch 1).

The synthesis was repeated to provide a second batch of Polymer A(2) (Batch 2).

#### Synthesis of Polymer B:

As in the Synthesis of Polymer A, a reaction solution of 50 494 grams of 1,3-dioxolane, 1.39 grams of methacrylamide, 15.98 grams of styrene, 21.80 grams of glycidyl methacrylate, and 0.83 grams of 1-dodecanethiol was formed.

TABLE II

| Compound              | Molar Ratio | Weight % | Amount (g) |
|-----------------------|-------------|----------|------------|
| Methacrylamide        | 5.00        | 3.48     | 1.39       |
| Styrene               | 46.875      | 39.94    | 15.98      |
| Glycidyl methacrylate | 46.875      | 54.51    | 21.80      |
| 1-Dodecanethiol       | 1.25        | 2.07     | 0.83       |

This reaction solution was stirred and warmed to reflux (about 65–70° C.) under a nitrogen sweep for one hour. 55 Then, 0.68 grams of a 5% (wt/wt) solution of AIBN dissolved in 1,3-dioxolane was added every hour for 20 hours. The reaction solution was then concentrated at ambient

## 17

pressure to approximately  $\frac{1}{3}$  to  $\frac{1}{5}$  volume and cooled. The resulting solution was poured with good stirring into cold methanol, collected, rinsed with cold methanol, collected, and dried at 40° C. at ambient pressure to collect Polymer B.

## Synthesis of Polymer C:

A reaction solution was formed as described above with 494 grams of 1,3-dioxolane, 2.83 grams of methacrylamide, 15.36 grams of styrene, 20.97 grams of glycidyl methacrylate, and 0.84 grams of 1-dodecanethiol.

TABLE III

| Compound              | Molar Ratio | Weight % | Amount (g) |
|-----------------------|-------------|----------|------------|
| Methacrylamide        | 10.00       | 7.07     | 2.83       |
| Styrene               | 44.375      | 38.41    | 15.36      |
| Glycidyl methacrylate | 44.375      | 52.42    | 20.97      |
| 1-Dodecanethiol       | 1.25        | 2.10     | 0.84       |

This reaction solution was stirred and warmed to reflux (about 65–70° C.) under a nitrogen sweep for one hour. Then 0.68 grams of a 5% (wt/wt) solution of AIBN dissolved in 1,3-dioxolane was added every hour for 20 hours. The reaction solution was concentrated at ambient pressure to approximately  $\frac{1}{3}$  to  $\frac{1}{5}$  volume then cooled. The resulting solution was poured with good stirring into cold methanol, collected, rinsed with cold methanol, collected, and dried at 40° C. at ambient pressure to collect Polymer C.

## Synthesis of Polymer D:

A reaction solution was formed with 353.5 g of propylene glycol methyl ether acetate, 22.0 g of glycidyl methacrylate, and 15.5 g of methyl methacrylate in a 1000 ml 4-neck ground glass flask, equipped with a heating mantle, temperature controller, mechanical stirrer, condenser, pressure equalized addition funnel and nitrogen inlet. The reaction mixture was heated to 80° C. under a nitrogen purge for one hour. After the nitrogen flow was changed and kept above the solution, 0.375 g of AIBN was added. A pre-mixture solution of 66.0 g of glycidyl methacrylate, 46.5 g of methyl methacrylate, and 0.75 g of AIBN was added over two hours at 80° C. The polymerization reaction was continued another seven hours during which 0.375 g of AIBN was added at intervals. The resulting Polymer D was obtained at >99% conversion based on a determination of % non-volatiles. The viscosity (G.H'33) was "T+" (~570 cps). Polymer D had a glycidyl methacrylate to methyl methacrylate weight ratio of 60:40.

## Synthesis of Polymer E:

A reaction mixture was formed with 235.6 g of propylene glycol methyl ether acetate, 20.0 g of glycidyl methacrylate,

and 5.0 g of methyl methacrylate in a 1000 ml 4-neck ground glass flask, equipped with a heating mantle, temperature controller, mechanical stirrer, condenser, pressure equalized addition funnel and nitrogen inlet. The reaction mixture was heated to 80° C. under a nitrogen purge for one hour. After the nitrogen flow was changed and kept above the solution, 0.25 g of AIBN was added. A pre-mixture solution of 60.0 g of glycidyl methacrylate, 15.0 g of methyl methacrylate, and 0.5 g of AIBN was added over two hours at 80° C. The polymerization reaction was continued another seven hours during which 0.25 g of AIBN was added at intervals. The resulting Polymer E was obtained at >99% conversion based on a determination of % non-volatiles. The viscosity (G.H'33) was "O" (~370 cps). Polymer E had a glycidyl methacrylate to methyl methacrylate weight ratio of 80:20

## Synthesis of Polymer F:

A reaction mixture was formed with 235.6 g of propylene glycol methyl ether acetate, 15.0 g of glycidyl methacrylate, 8.7 g of methyl methacrylate, and 1.2 g of t-butyl acrylate in a 1000 ml 4-neck ground glass flask, equipped with a heating mantle, temperature controller, mechanical stirrer, condenser, pressure equalized addition funnel and nitrogen inlet. The reaction mixture was heated to 80° C. under a nitrogen purge for one hour. After the nitrogen flow was changed and kept above the solution, 0.25 g of AIBN was added. A pre-mixture of 45.0 g of glycidyl methacrylate, 26.3 g of methyl methacrylate, 3.8 g of t-butyl acrylate, and 0.5 g of AIBN were added in two hours at 80° C. The polymerization reaction was continued another eight hours, during which 0.5 g of AIBN was added at intervals. The Polymer F conversion was >99% based on determination of percent of non-volatiles. The viscosity (G.H'33) was "O" (~370 cps). Polymer F had a glycidyl methacrylate, methyl methacrylate, and t-butyl acrylate weight ratio of 60:35:5.

## Examples 1–6

Imageable elements containing the various epoxy-containing polymers described herein in the outer (top) layer were prepared as follows:

Inner layer formulations were prepared with the components described in TABLE IV below and applied to Substrate A using a 0.012 inch (0.03 cm) wire-wound bar and dried for 30 seconds at 135° C. to provide a dry coated film of approximately 1.5 g/cm<sup>2</sup>.

Topcoat (outer layer) solutions were prepared with the components described in TABLE V below and applied with a 0.006 inch (0.015 cm) wire-wound bar and dried at 30 seconds at 135° C. to provide a dry coat weight of approximately 0.60 g/cm<sup>2</sup>.

TABLE IV

## Inner Layer Formulations Based on 80 g of Coating Solution with 7.0% Non-volatiles

|               | BYK307<br>10% solution |         |          |          |          |        |          |
|---------------|------------------------|---------|----------|----------|----------|--------|----------|
|               | JK69                   | ACR1478 | IR Dye A | IR Dye B | IR Dye C | in DEK | Solvent* |
| Inner Layer A | 4.556                  | 0       | 0.560    | 0        | 0.450    | 0.364  | 74.072   |
| Inner Layer B | 0                      | 4.556   | 0        | 0.560    | 0.450    | 0.364  | 74.072   |

\*Solvent mixture - MEK/PGME/BLO/water 50/30/10/10 by weight.

TABLE V

Upper Layer Formulations Based on 25 g of Coating Solution with 6.0% Non-volatiles

|               | Polymer A(1) | Polymer A(2) | Polymer D | Polymer E | Ethyl violet 1% solution in acetone | BYK307 10% solution In DEK | Solvent X* | Solvent Y* | Polymer F 30% solution in PGMEA |
|---------------|--------------|--------------|-----------|-----------|-------------------------------------|----------------------------|------------|------------|---------------------------------|
| Outer Layer A | 1.485        | 0            | 0         | 0         | 0.525                               | 0.100                      | 22.890     | 0          | 0                               |
| Outer Layer B | 0            | 0            | 1.485     | 0         | 0.525                               | 0.100                      | 22.890     | 0          | 0                               |
| Outer Layer C | 0            | 0            | 0         | 1.485     | 0.525                               | 0.100                      | 22.890     | 0          | 0                               |
| Outer Layer D | 1.485        | 0            | 0         | 0         | 0.300                               | 0.120                      | 0          | 23.095     | 0                               |
| Outer Layer E | 0            | 1.485        | 0         | 0         | 0.300                               | 0.120                      | 0          | 23.095     | 0                               |
| Outer Layer F | 0            | 0            | 0         | 0         | 0.300                               | 0.120                      | 0          | 19.630     | 4.950                           |

\*Solvent X mixture - PGMEA/DEK/PGMEA (30:62:8 weight ratio)

\*Solvent Y mixture - DEK/PGMEA (92:8 weight ratio)

The imageable elements were then subjected to the following tests:

#### Developer Solubility:

Drops of a developer solution of water and TSD01 (5:1 v/v) were applied to the each element at 10-second intervals for 180 seconds. The developer solution was washed off immediately with water. The time required for surface (upper layer) deterioration to begin (in seconds) was recorded.

#### Imaging Tests:

Each element was imaged using a commercially available Screen PlateRite 4300 series platesetter. A C1 2400Dpi internal test pattern was applied at a drum speed of 1000 rpm using exposures of 50, 55, 60, 65, 70, 75, 80, 85 & 90% power. The resulting imaged printing plates were processed in a Kodak Polychrome Graphics PK910II processor containing a developer solution of water and TSD01 (5:1 v/v) at 30° C. for 12 seconds. The developed plates were then evaluated for cleanout (that is, the minimum exposure necessary to produce a clean image) and best exposure (that is, the exposure that produces the best image quality).

All of the elements had upper layers that exhibited good resistance to the developer solution and that produced high quality images after exposure and development. The detailed results are provided below in TABLE VI.

TABLE VI

| Example | Inner Layer | Outer Layer | Developer Test | Cleanout Energy | Best Exposure | Comments                       |
|---------|-------------|-------------|----------------|-----------------|---------------|--------------------------------|
| 1       | A           | A           | >180           | 85              | 90            | Image had excellent resolution |
| 2       | A           | B           | >180           | 85              | 90            | Image had good resolution      |
| 3       | A           | C           | >180           | 85              | 90            | Image had good resolution      |
| 4       | B           | D           | 40             | 70              | 75            | Image had excellent resolution |
| 5       | B           | E           | 50             | 65              | 70            | Image had excellent resolution |
| 6       | A           | F           | >180           | 75              | 90            | Image had good resolution      |

## Comparative Examples 1 and 2

Imageable element was prepared, imaged, and evaluated similarly to the imageable elements described in Examples 1–6 except that the outer layer of these comparative elements contained a hardened epoxy-containing polymer according to the teaching in U.S. Pat. No. 6,152,036 (noted above). The layer formulations are described in the following TABLE VII.

TABLE VII

|                                                                       |                                                       |                              |                        |           |
|-----------------------------------------------------------------------|-------------------------------------------------------|------------------------------|------------------------|-----------|
| 20                                                                    | Inner Layer Formulation - % of total dry layer weight |                              |                        |           |
| JK69                                                                  | IR Dye B                                              | IR Dye C                     | Byk ® 307              |           |
| 81.35                                                                 | 10                                                    | 8                            | 0.65                   |           |
| 25 Inner Layer Formulation based on 50 g coating solution (7% solids) |                                                       |                              |                        |           |
| JK69                                                                  | IR Dye B                                              | IR Dye C                     | Byk ® 307<br>(10% DEK) | Solvent*  |
| 2.847                                                                 | 0.350                                                 | 0.280                        | 0.228                  | 46.295    |
| 30 Outer Layer Formulation - % total layer dry weight                 |                                                       |                              |                        |           |
| Epon 1001F                                                            | 2-Methyl-imidazole                                    | Ethyl Violet                 | Byk ® 307              |           |
| 91.00                                                                 | 8.00                                                  | 0.20                         | 0.8                    |           |
| 35 Topcoat formulation based on 25 g coating solution at 6% solids    |                                                       |                              |                        |           |
| Epon 1001F                                                            | 2-Methyl-imidazole                                    | Ethyl Violet<br>(1% acetone) | Byk ® 307<br>(10% DEK) | Solvent** |
| 1.365                                                                 | 0.120                                                 | 0.300                        | 0.120                  | 23.095    |

\*solvent = Methyl ethyl ketone/methyl lactate/butyrolactone/water (50/30/10/10)

\*\*Solvent = Diethyl ketone/propylene glycol methyl ether acetate (92/8)

## Comparative Example 1

60 The inner layer formulation was applied to Substrate A using a 0.012 inch (0.03 cm) wire-wound bar to provide a dry coating film of approximately 1.5 g/m<sup>2</sup>. The resulting layer was dried for 30 seconds at 135° C. after which the outer layer formulation was applied using a 0.006 inch (0.015 cm) wire-wound bar to provide a dry coating weight of approximately 0.60 g/m<sup>2</sup>. This outer layer was dried for 40 seconds at 135° C.

## 21

Samples of the imageable elements were subject to the following tests:

Developer solubility: Drops of water/TSD01 (4:1) were applied to the element samples at 10-second intervals for up to 120 seconds, and the developer was washed off immediately with water. The time taken for the developer to start attacking the outer was recorded.

Imaging tests: Element samples were imaged with a Screen PTR4300. The C1 2400 Dpi internal test pattern was applied at a drum speed of 1000 rpm with exposures of 50, 55, 60, 65, 70, 75, 80, 85 & 90% power. The imaged elements were processed in a Kodak Polychrome Graphics PK910II processor containing water/TSD01 (4:1) at a developer temperature of 30° C. and a development time of 12 seconds. Imaged and developed element samples were then evaluated for cleanout (minimum exposure necessary to produce a clean image) and best exposure (the exposure which produces best image quality). The results are shown below in TABLE VIII.

## Comparative Example 2

Imageable elements were prepared and evaluated as described in Comparative Example 1 except that the outer layer formulation was dried for 60 seconds at ~160° C. The test results are shown below in TABLE VIII.

TABLE VIII

| Comparative Example | Developer Drop Test | Cleanout Energy | Best Exposure | Comments                                         |
|---------------------|---------------------|-----------------|---------------|--------------------------------------------------|
| 1                   | <10 sec             | —               | —             | Layers washed away                               |
| 2                   | >>120 sec           | —               | —             | Inner Layer washed away but Outer Layer remained |

These results show that the Comparative imageable elements were unacceptable in performance. The elements of Comparative Example 1 exhibited poor resistance to the developer in the unexposed regions (they were washed away during development). Thus, a useful printing image could not be obtained (hence, cleanout energy and best exposure could not be evaluated).

The elements of Comparative Example 2 exhibited excellent resistance to the developer, suggesting that hardening of the outer layer resin had been achieved. After imaging and processing a good image was obtained. However, upon further inspection, it was discovered that the inner layer had been washed away in the exposed areas, but the outer layer had not been removed and remained on the substrate. Since the outer layer was ink receptive, a useful printing image was not obtained (hence, cleanout energy and best exposure could not be evaluated).

The invention has been described in detail with particular reference to certain preferred embodiments thereof, but it will be understood that variations and modifications can be effected within the spirit and scope of the invention.

The invention claimed is:

1. A positive-working imageable element comprising a radiation absorbing compound, and a substrate having thereon, in order:
  - an inner layer comprising a polymeric material that is removable using an alkaline developer, and
  - an ink receptive outer layer that is not removable using an alkaline developer before its exposure to imaging radia-

## 22

tion, that comprises a polymer binder having pendant epoxy groups sufficient to provide an epoxy equivalent weight of at from about 130 to about 1000, and that is free of hardener for said pendant epoxy groups.

2. The element of claim 1 wherein said outer layer polymer binder has pendant epoxy groups sufficient to provide an epoxy equivalent weight of from about 140 to about 750.
3. The element of claim 1 wherein said polymer binder having pendant epoxy groups is present in said outer layer in a dry coverage of from about 20 to about 99.9 weight % based on total dry weight of said outer layer.
4. The element of claim 1 wherein said outer layer polymer binder is an acrylic resin derived from one or more ethylenically unsaturated polymerizable monomers, at least one of which monomers comprises pendant epoxy groups.
5. The element of claim 4 wherein said outer layer polymeric binder having pendant epoxy groups is represented by the following Structure (I):

20



30 wherein R<sup>1</sup> is hydrogen, an alkyl group having 1 to 6 carbon atoms, or a halo group, R<sup>2</sup> represents a group containing an epoxy moiety, L is a direct bond or a linking group, B represents recurring units derived from one or more ethylenically unsaturated polymerizable monomers that do not have pendant epoxy groups, x is from about 20 to 100 weight %, and y is from 0 to about 80 weight %.

6. The element of claim 5 wherein R<sup>1</sup> is hydrogen, methyl, or chloro, L is —C(O)O-alkylene, —C(O)O-alkylene-phenylene-, or —C(O)O-phenylene, wherein alkylene has 1 to 4 carbon atoms, x is from about 40 to about 95 weight %, y is from about 5 to about 60 weight %, and R<sup>2</sup> is a glycidyl or 3,4-epoxycyclohexyl group.

7. The element of claim 5 wherein B represents recurring units derived from one or more (meth)acrylate, (meth)45 acrylamide, vinyl ether, vinyl ester, vinyl ketone, olefin, unsaturated imide, N-vinyl pyrrolidone, N-vinyl carbazole, vinyl pyridine, (meth)acrylonitrile, or styrenic monomers.

8. The element of claim 5 wherein x is from about 40 to 95 weight % and the recurring units comprising pendant epoxy groups are derived from one or more of glycidyl acrylate, glycidyl methacrylate, 3,4-epoxycyclohexyl methacrylate, and 3,4-epoxycyclohexyl acrylate.

9. The element of claim 1 wherein said polymer binder has from about 50 to about 80 weight % of recurring units 55 that are derived from one or more of glycidyl acrylate, glycidyl methacrylate, 3,4-epoxycyclohexyl methacrylate, and 3,4-epoxycyclohexyl acrylate, and at least some recurring units derived from one or more styrenic monomers.

10. The element of claim 9 wherein said polymer binder comprises B recurring units that are derived from styrene.

11. The element of claim 1 wherein said infrared radiation absorbing compound is a carbon black or IR absorbing dye having a maximum absorption at from about 800 to about 1200 nm and is present in said inner layer in an amount of at least 12 weight %.

12. The element of claim 1 wherein said outer layer further comprises a colorant, a coating surfactant, or both.

23

13. The element of claim 1 wherein said inner layer polymeric material is a polyvinyl acetal, a (meth)acrylic resin comprising carboxy groups, a vinyl acetate-crotonate-vinyl neodecanoate copolymer phenolic resin, a maleated wood rosin, a styrene-maleic anhydride copolymer, a (meth)acrylamide polymer, a polymer derived from an N-substituted cyclic imide, or a combination thereof.

14. The element of claim 1 wherein said inner layer polymeric material is a polyvinyl acetal or a copolymer derived from an N-substituted cyclic imide, a methacrylamide, and (meth)acrylic acid.

15. The element of claim 13 wherein said inner layer further comprises an additional polymeric material that is a novolak or resole resin.

16. The element of claim 1 wherein said inner layer has a dry coating weight of from about 0.5 to about 2.5 g/m<sup>2</sup> and said outer layer has a dry coating weight of from about 0.2 to about 1 g/m<sup>2</sup>.

17. A method for forming an image comprising:

A) thermally imaging a positive-working imageable element comprising a radiation absorbing compound and a substrate having thereon, in order:

an inner layer comprising a polymeric material that is removable using an alkaline developer, and an ink receptive outer layer that is not removable using an alkaline developer before its exposure to imaging radiation, that comprises a polymer binder having pendant epoxy groups sufficient to provide an epoxy equivalent weight of from about 130 to about 1000, thereby forming an imaged element with imaged and non-imaged regions, and

B) contacting said imaged element with an alkaline developer to remove only said imaged regions, and

C) optionally, baking said imaged and developed element, wherein the imaged element obtained in step A is characterized wherein the pendant epoxy groups in said polymer binder of said outer layer are substantially unreacted.

18. The method of claim 17 wherein said developer comprises a thiosulfate salt or an amino compound having at

24

least one N-hydrogen atom and an alkyl group that is substituted with a hydroxy or acidic group or a polyethylene oxide chain.

19. The method of claim 17 wherein imaging in step A is carried out using infrared radiation in the range of from about 800 nm to about 1120 nm.

20. The method of claim 17 wherein said outer layer polymeric binder having pendant epoxy groups is represented by the following Structure (I):



wherein R<sup>1</sup> is hydrogen or methyl, R<sup>2</sup> is a glycidyl or 3,4-epoxycyclohexyl group, L is —C(O)O-alkylene, —C(O)O-alkylene-phenylene-, or —C(O)O-phenylene, wherein alkylene has 1 to 4 carbon atoms, x is from about 40 to about 95 weight %, y is from about 5 to about 60 weight %,

B represents recurring units derived from one or more (meth)acrylate, (meth)acrylamide, vinyl ether, vinyl ester, vinyl ketone, olefin, unsaturated imide, N-vinyl pyrrolidone, N-vinyl carbazole, vinyl pyridine, (meth)acrylonitrile, or styrenic monomers,

said inner layer comprises said radiation absorbing compound that is an IR absorbing dye, and

said inner layer polymeric material is a polyvinyl acetal, or a copolymer derived from an N-substituted cyclic imide, a methacrylamide, and a (meth)acrylic acid.

21. An image obtained from the method of claim 17.

\* \* \* \* \*